

# United States Patent [19]

Yagihara et al.

[11] Patent Number: 4,474,870

[45] Date of Patent: Oct. 2, 1984

[54] SILVER HALIDE COLOR PHOTOGRAPHIC LIGHT-SENSITIVE MATERIAL

[75] Inventors: Morio Yagihara; Keiji Miayashi; Takashi Ozawa, all of Kanagawa, Japan

[73] Assignee: Fuji Photo Film Company Limited, Kanagawa, Japan

[21] Appl. No.: 457,318

[22] Filed: Jan. 11, 1983

[30] Foreign Application Priority Data

Jan. 11, 1982 [JP] Japan 57-2419

[51] Int. Cl.<sup>3</sup> G03C 7/16; G03C 7/26

[52] U.S. Cl. 430/381; 430/386; 430/548; 430/554

[58] Field of Search 430/548, 381, 386, 387, 430/554, 555

[56] References Cited

U.S. PATENT DOCUMENTS

4,080,211 3/1978 Paesschen et al. 430/548  
4,340,664 7/1982 Monbaliu et al. 430/548  
4,367,282 1/1983 Yagihara et al. 430/381  
4,388,404 6/1983 Morigaki et al. 430/555

Primary Examiner—J. Travis Brown  
Attorney, Agent, or Firm—Sughrue, Mion, Zinn,  
Macpeak and Seas

[57] ABSTRACT

A silver halide color photographic light-sensitive material comprising a support having thereon a silver halide emulsion layer containing a magenta color image forming polymer coupler latex which is capable of forming a dye upon coupling with an oxidation product of an aromatic primary amine developing agent and which is a polymer or copolymer having a repeating unit derived

from a monomer represented by the following general formula (I):



wherein R<sub>1</sub> represents a hydrogen atom, a lower alkyl group containing from 1 to 4 carbon atoms or a chlorine atom; R<sub>2</sub> represents an unsubstituted or substituted alkylene group which may be a straight chain or a branched chain; R<sub>3</sub> represents an unsubstituted or substituted alkylene group which may be a straight chain or a branched chain, an unsubstituted or substituted phenylene group or an unsubstituted or substituted aralkylene group; X represents —CONH—, —NHCONH— or —NHCOO—; Y represents —CONH— or —COO—; Z represents —O—, —S—, —SO—, —SO<sub>2</sub>—, —CONH— or —COO—; Ar represents an unsubstituted or substituted phenyl group; l represents 0 or 1; m represents 0 or 1; and n represents 0 or 1.

The magenta color image forming polymer coupler latex has a good color forming property and is capable of forming a dye with a high yield and without formation of undesired stains and fogs, and the silver halide color photographic light-sensitive material containing the magenta color image forming polymer coupler latex has good film strength and a reduced layer thickness and provides a stable magenta image having an improved sharpness and a good fastness to light, heat, and humidity. A method of forming a color image using the silver halide color photographic light-sensitive material is also described.

21 Claims, No Drawings

## SILVER HALIDE COLOR PHOTOGRAPHIC LIGHT-SENSITIVE MATERIAL

### FIELD OF THE INVENTION

The present invention relates to a silver halide color photographic light-sensitive material containing a novel magenta color image forming polymer coupler latex capable of coupling with an oxidation product of an aromatic primary amine developing agent.

### BACKGROUND OF THE INVENTION

It is well known that for the color development of a silver halide photographic light-sensitive material, after exposure, an oxidized aromatic primary amine developing agent can be reacted with a dye forming coupler to obtain a color image.

It is also known that, for the color development of a silver halide color photographic material, an oxidized aromatic primary amine color developing agent can be reacted with a coupler to form a dye such as an indo-phenol, an indoaniline, an indamine, an azomethine, a phenoxazine, a phenazine, and the like, thus forming a color image. In this procedure, the subtractive color process is ordinarily used for color reproduction, and silver halide emulsions which are selectively sensitive to blue, green and red light, and yellow, magenta and cyan color image formers, which are respectively the complementary colors of blue, green and red, are employed. For example, a coupler of the acylacetanilide or benzoylmethane type is used for forming a yellow color image; a coupler of the pyrazolone, pyrazolobenzimidazole, cyanoacetophenone or indazolone type is generally used for forming a magenta color image; and a phenolic coupler, such as phenols and naphthols, is generally used for forming a cyan color image.

Color couplers must satisfy various requirements. For example, it is necessary that they have a good spectral property and provide a dye image having excellent stability to light, temperature, and humidity for a long period of time upon color development.

It is also required in a multilayer color photographic light-sensitive material that couplers are fixed in respective layers separated from each other in order to reduce color mixing and improve color reproduction. Many methods for rendering a coupler diffusion-resistant are known. One method is to introduce a long chain aliphatic group into a coupler molecule in order to prevent diffusion. Couplers according to such a method require a step of addition to an aqueous gelatin solution by solubilizing in alkali, or a step of dispersing in an aqueous gelatin solution by dissolving in a high boiling point organic solvent, since the couplers are immiscible with an aqueous gelatin solution. Such color couplers may cause crystal formation in a photographic emulsion. Furthermore, when using a high boiling point organic solvent, a large amount of gelatin must be employed since the high boiling point organic solvent makes an emulsion layer soft. Consequently, this increases the thickness of the material even though it is desirable to reduce the thickness of the emulsion layer.

Another method for rendering a coupler diffusion-resistant is to utilize a polymer coupler latex obtained by polymerization of a monomeric coupler. An example of a method of adding a polymer coupler in a latex form to a hydrophilic colloid composition is a method in which a latex prepared by an emulsion polymerization method is directly added to a gelatino silver halide emulsion and

a method in which an oleophilic polymer coupler obtained by polymerization of a monomeric coupler is dispersed in a latex form in an aqueous gelatin solution. Some examples of the former emulsion polymerization methods include an emulsion polymerization method in an aqueous gelatin phase as described in U.S. Pat. No. 3,370,952 and an emulsion polymerization method in water as described in U.S. Pat. No. 4,080,211. An example of the latter method in which a lipophilic polymer coupler is dispersed in a latex form in gelatin is described in U.S. Pat. No. 3,451,820. The method of adding a polymer coupler in a latex form to a hydrophilic colloid composition has many advantages in comparison with other methods. For example, the deterioration of strength of the film formed is small, because the hydrophobic substance is in a latex form. Also, since the latex can contain coupler monomers in a high concentration, it is easy to incorporate couplers in a high concentration into a photographic emulsion, and the increase of viscosity is small. Furthermore, color mixing is prevented, since a polymer coupler is completely immobilized and the crystallization of couplers in the emulsion layer is small. In particular, when the polymer coupler latex prepared by an emulsion polymerization method is used, the step of adding the coupler to a coating solution can be simplified, since the use of a high boiling point organic solvent or an alkali is not necessary and a special dispersing method is not required. Moreover, the thickness of the layer can be reduced, since an organic solvent is not contained therein.

With respect to the addition of these polymer couplers in a latex form to a gelatino silver halide emulsion, there are described, for example, 4-equivalent magenta polymer coupler latexes and methods of preparation thereof in U.S. Pat. No. 4,080,211, British Pat. No. 1,247,688, and U.S. Pat. No. 3,451,820, copolymer latexes with a competing coupler in West German Pat. No. 2,725,591, and U.S. Pat. No. 3,926,436 and cyan polymer coupler latexes in U.S. Pat. No. 3,767,412.

However, these polymer coupler latexes have a number of problems which need to be eliminated, in addition to the many advantages described above. The problems include the following:

1. The absorption peak of the magenta dye is broadened, and thus the color reproducibility is inferior.
2. The rate of the coupling reaction is poor, and thus the density of dye formed is very low.
3. The light fastness of the magenta color image is very poor.
4. Undesirable fog is readily formed upon color development.
5. The fastness to humidity and heat of the color image is poor.
6. The solubility of the coupler monomer is low, and the polymerizability thereof is very poor.

More particularly, they have major disadvantages in color reproducibility, coupling reactivity, light fastness of magenta color image, stability of polymer coupler latex in a film during storage, and the polymerizability of the coupler monomer. With respect to the coupling reactivity, no improvement is obtained by using the 2-equivalent magenta polymer coupler latex described in West German Pat. No. 2,725,591 and U.S. Pat. No. 3,926,436. This suggests that there are great differences in photographic properties between conventional couplers and polymer couplers.

## SUMMARY OF THE INVENTION

An object of the present invention is to provide a novel magenta color image forming polymer coupler latex in which the disadvantages described above are eliminated, and which is free from the formation of undesirable fog and stain.

Another object of the present invention is to provide a novel magenta color image forming polymer coupler latex which has an excellent color forming property.

Another object of the present invention is to provide a novel magenta color image forming polymer coupler latex which provides an excellent color reproducibility.

Still another object of the present invention is to provide a color photographic light-sensitive material that forms a color image fast to light, heat, and humidity in a color photograph after development processing.

A further object of the present invention is to provide a color photographic light-sensitive material having good film strength.

A further object of the present invention is to provide a color photographic light-sensitive material having a reduced layer thickness and an improved sharpness.

A still further object of the present invention is to provide a method of forming a magenta color image by development of a silver halide emulsion in the presence of a novel magenta dye forming polymer coupler latex.

A still further object of the present invention is to provide a silver halide color photographic light-sensitive material containing a novel magenta dye forming polymer coupler latex, a photographic processing method or an image forming method for using the material.

Other objects of the present invention will be apparent from the following detailed description and examples.

As a result of extensive investigations, it has now been found that these objects of the present invention are accomplished by the use of a magenta color image forming polymer coupler latex which is a polymer or copolymer having a repeating unit derived from a monomer represented by the following general formula (I):



wherein  $\text{R}_1$  represents a hydrogen atom, a lower alkyl group containing from 1 to 4 carbon atoms or a chlorine atom;  $\text{R}_2$  represents an unsubstituted or substituted alkylene group which may be a straight chain or a branched chain;  $\text{R}_3$  represents an unsubstituted or substituted alkylene group which may be a straight chain or a branched chain, an unsubstituted or substituted phenylene group or an unsubstituted or substituted aralkylene group;  $\text{X}$  represents  $-\text{CONH}-$ ,  $-\text{NHCONH}-$  or  $-\text{NHCOO}-$ ;  $\text{Y}$  represents  $-\text{CONH}-$  or  $-\text{COO}-$ ;  $\text{Z}$  represents  $-\text{O}-$ ,  $-\text{S}-$ ,  $-\text{SO}-$ ,  $-\text{SO}_2-$ ,  $-\text{CONH}-$  or  $-\text{COO}-$ ;  $\text{Ar}$  represents an unsubstituted or substituted phenyl group;  $\text{l}$  represents 0 or 1;  $\text{m}$  represents 0 or 1; and  $\text{n}$  represents 0 or 1.

In more detail, the objects of the invention can be accomplished with a color photographic light-sensitive

material comprising a support having thereon at least one silver halide emulsion layer containing a magenta color image forming polymer coupler latex which is a novel polymer having a repeating unit represented by the general formula (II) described below, or a novel copolymer of the repeating unit described below and a non-color forming unit which does not couple with the oxidation product of an aromatic primary amine developing agent.

10



20

wherein  $\text{R}_1$ ,  $\text{R}_2$ ,  $\text{R}_3$ ,  $\text{X}$ ,  $\text{Y}$ ,  $\text{Z}$ ,  $\text{Ar}$ ,  $\text{l}$ ,  $\text{m}$  and  $\text{n}$  have the same meanings as defined in the general formula (I) above.

## DETAILED DESCRIPTION OF THE INVENTION

The novel magenta color image forming polymer coupler latex according to the present invention includes a polymer having a repeating unit derived from a monomer coupler represented by the general formula (I), and a copolymer of the repeating unit according to formula (II) and at least one non-color forming unit containing at least one ethylene group which does not have an ability of oxidative coupling with an aromatic primary amine developing agent.

In the above-described formula (I),  $\text{R}_1$  represents a hydrogen atom, a lower alkyl group having from 1 to 4 carbon atoms, or a chlorine atom;  $\text{R}_2$  represents an unsubstituted or substituted alkylene group, preferably having from 1 to 10 carbon atoms, which may be a straight chain or a branched chain;  $\text{R}_3$  represents an unsubstituted or substituted alkylene group, preferably having from 1 to 10 carbon atoms, which may be a straight chain or a branched chain, an unsubstituted or substituted phenylene group or an unsubstituted or substituted aralkylene group. Examples of the alkylene group for  $\text{R}_2$  and  $\text{R}_3$  include a methylene group, a methylmethylen group, a dimethylmethylen group, a trimethylmethylen group, a tetramethylmethylen group, a pentamethylmethylen group, a decylmethylmethylen group, etc. Examples of the phenylene group for  $\text{R}_3$  include a p-phenylene group, an m-phenylene group, a methylphenylene group, etc.

$\text{X}$  represents  $-\text{CONH}-$ ,  $-\text{NHCONH}-$  or  $-\text{NHCOO}-$ ;  $\text{Y}$  represents  $-\text{CONH}-$  or  $-\text{COO}-$ ;  $\text{Z}$  represents  $-\text{O}-$ ,  $-\text{S}-$ ,  $-\text{SO}-$ ,  $-\text{SO}_2-$ ,  $-\text{CONH}-$  or  $-\text{COO}-$ ;  $\text{Ar}$  represents an unsubstituted or substituted phenyl group;  $\text{l}$  represents 0 or 1;  $\text{m}$  represents 0 or 1; and  $\text{n}$  represents 0 or 1.

Substituents for the alkylene group, the phenylene group or the aralkylene group represented by  $\text{R}_2$  or  $\text{R}_3$  include an aryl group (for example, a phenyl group, etc.), a nitro group, a hydroxy group, a cyano group, a sulfo group, an alkoxy group (for example, a methoxy group, etc.), an aryloxy group (for example, a phenoxy group, etc.), an acyloxy group (for example, an acetoxy group, etc.), an acylamino group (for example, an

acetylamino group, etc.), a sulfonamido group (for example, a methanesulfonamido group, etc.), a sulfamoyl group (for example a methylsulfamoyl group, etc.), a halogen atom (for example, a fluorine atom, a chlorine atom, a bromine atom, etc.), a carboxy group, a carbamoyl group (for example, a methylcarbamoyl group, etc.), an alkoxy carbonyl group (for example, a methoxycarbonyl group, etc.), a sulfonyl group (for example, a methylsulfonyl group, etc.), and the like. When two or more substituents are present, they may be the same or different.

Ar represents an unsubstituted or substituted phenyl group. Substituents for the phenyl group include an alkyl group (for example, a methyl group, an ethyl group, etc.), an alkoxy group (for example, a methoxy group, an ethoxy group, etc.), an aryloxy group (for example, a phenoxy group, etc.), an alkoxy carbonyl group (for example, a methoxycarbonyl group, etc.), an acylamino group (for example, an acetylamino group, etc.), a carbamoyl group, an alkylcarbamoyl group (for example, a methylcarbamoyl group, an ethylcarbamoyl group, etc.), a dialkylcarbamoyl group (for example, a dimethylcarbamoyl group, etc.), an arylcarbamoyl group (for example, a phenylcarbamoyl group, etc.), an alkylsulfonyl group (for example, a methylsulfonyl group, etc.), an arylsulfonyl group (for example, a phenylsulfonyl group, etc.), an alkylsulfonamido group (for example, a methanesulfonamido group, etc.), an arylsulfonamido group (for example, a phenylsulfonamido group, etc.), a sulfamoyl group, an alkylsulfamoyl group (for example, an ethylsulfamoyl group, etc.), a dialkylsulfamoyl group (for example, a dimethylsulfamoyl group, etc.), an alkylthio group (for example, a methylthio group, etc.), an arylthio group (for example, a phenylthio group, etc.), a cyano group, a nitro group, a halogen atom (for example, a fluorine atom, a chlorine atom, a bromine atom, etc.), and the like. When two or more substituents are present, they may be the same or different.

Particularly preferred substituents for Ar include a halogen atom, an alkyl group, an alkoxy group, an alkoxy carbonyl group and a cyano group.

Of the substituted phenyl groups represented by Ar, preferred groups are those represented by the following general formula (III):



wherein R<sub>4</sub>, which is present at the 4-position or 5-position of the phenyl group, represents a halogen atom (for example, a fluorine atom, a chlorine atom, a bromine atom, etc.), an acylamino group (for example, an acetylamino group, etc.), a carbamoyl group (for example, a carbamoyl group, a methylcarbamoyl group, a dimethylcarbamoyl group, etc.), a sulfonyl group (for example, a methylsulfonyl group, etc.), a sulfonamido group (for example, a methanesulfonamido group, etc.), a cyano group or an alkoxy carbonyl group (for example, a methoxycarbonyl group, an ethoxycarbonyl group, etc.). Of these substituents represented by R<sub>4</sub>, a halogen atom is particularly preferred in view of color reproducibility, color forming property and stability.

Examples of the non-color forming monomer which does not couple with the oxidation product of an aromatic primary amine developing agent include an ester, preferably a lower alkyl ester, and an amide, derived from an acrylic acid, for example, an acrylic acid, an  $\alpha$ -chloroacrylic acid, an  $\alpha$ -alkylacrylic acid such as a methacrylic acid (for example, acrylamide, methacrylamide, t-butylacrylamide, methyl acrylate, methyl methacrylate, ethyl acrylate, n-propyl acrylate, isopropyl acrylate, n-butyl acrylate, sec-butyl acrylate, t-butyl acrylate, n-butyl methacrylate, 2-ethylhexyl acrylate, n-hexyl acrylate, n-octyl methacrylate, lauryl acrylate, methylenebisacrylamide, etc.), a vinyl ester (for example, vinyl acetate, vinyl propionate, vinyl laurate, etc.), acrylonitrile, methacrylonitrile, an aromatic vinyl compound, for example, styrene and a derivative thereof, for example, vinyl toluene, divinyl benzene, vinyl acetophenone, sulfostyrene, etc., itaconic acid, citraconic acid, crotonic acid, vinylidene chloride, a vinyl alkyl ether, for example, vinyl ethyl ether, an ester of maleic acid, N-vinyl-2-pyrrolidone, N-vinylpyridine, 2- or 4-vinylpyridine, etc.

Of these monomers, an ester of acrylic acid, an ester of methacrylic acid, an ester of maleic acid are particularly preferred.

Two or more comonomer compounds described above can be used together. For example, a combination of n-butyl acrylate and divinyl benzene, styrene and methacrylic acid, n-butyl acrylate and methacrylic acid, etc., can be used.

The ethylenically unsaturated monomer which is used to copolymerize with the monomer coupler represented by the above-described general formula (I) can be selected so that the copolymer to be formed possesses good physical properties and/or chemical properties, for example, solubility, compatibility with a binder such as gelatin in a photographic colloid composition, flexibility, heat stability, etc., as well known in the field of polymer color couplers.

The magenta polymer coupler latex used in the present invention can be prepared by an emulsion polymerization method as described above, or by dissolving an oleophilic polymer coupler obtained by polymerization of a monomer coupler in an organic solvent and then dispersing the solution in a latex form in an aqueous gelatin solution. With respect to the emulsion polymerization, the methods as described in U.S. Pat. Nos. 4,080,211 and 3,370,952 and with respect to the method in which an oleophilic polymer coupler is dispersed in a latex form in an aqueous gelatin solution, the method as described in U.S. Pat. No. 3,451,820 can be employed, respectively. These methods can be applied to both the preparation of homopolymers and copolymers. In the latter case, a non-color forming comonomer is preferably a liquid comonomer which may act, in the case of the emulsion polymerization, as a solvent for a monomer which is normally solid.

Free radical polymerization of an ethylenically unsaturated solid monomer is initiated with the addition to the monomer molecule of a free radical which is formed by thermal decomposition of a chemical initiator, an action of a reducing agent to an oxidative compound (a redox initiator) or a physical action, for example, irradiation of ultraviolet rays or other high energy radiations, high frequencies, etc.

Examples of the chemical initiators commonly used include a water-soluble initiator, for example, a persulfate (such as ammonium persulfate, potassium persulfate,

fate, etc.), hydrogen peroxide, 4,4'-azobis(4-cyanovaleric acid), etc., and a water-insoluble initiator, for example, azobisisobutyronitrile (such as 2,2'-azobis(2,4-dimethylvaleronitrile), 2,2'-azobisisobutyronitrile, etc.), benzoyl peroxide, chlorobenzoyl peroxide, and other compounds. Examples of the redox initiators usually used include hydrogen peroxide-iron (II) salt, potassium persulfate-potassium hydrogensulfate, cerium salt-alcohol, etc. Specific examples and functions of the initiators are described in F. A. Bovey, *Emulsion Polymerization*, pages 59-93, (Interscience Publisher Inc., New York (1955)).

The emulsifier which can be used in the emulsion polymerization may be a compound having surface activity. Preferred examples include soap, a sulfonate, a sulfate, a cationic compound, an amphoteric compound and a high molecular weight protective colloid. Specific examples and functions of the emulsifiers are described in *Belgische Chemische Industrie*, Vol. 28, pages 16-20 (1963).

On the other hand, an organic solvent which is used for dissolving an oleophilic polymer coupler when the oleophilic polymer coupler is dispersed in a latex form in an aqueous gelatin solution is removed from the mixture before coating of the dispersion solution or by 15 vaporization during drying of the dispersion solution coated, although the latter is less preferable. With respect to removing the solvent, a method in which the solvent is removed by washing a gelatin noodle with water is applied when the solvent is water-soluble to 20 some extent, or a spray drying method, a vacuum purging method or a steam purging method can be employed for removing the solvent.

Examples of the organic solvents which can be removed include, for example, an ester (for example, a 35 lower alkyl ester, etc.), a lower alkyl ether, ketone, halogenated hydrocarbon (for example, methylene chloride, trichloroethylene, a fluorinated hydrocarbon, etc.), an alcohol (for example, an alcohol between n-butyl alcohol and octyl alcohol, etc.), and a mixture 40 thereof.

Any type of dispersing agent can be used in the dispersion of the oleophilic polymer coupler. Ionic surface active agents, and particularly anionic surface active agents are preferred. Amphoteric surface active agents 45 such as C-cetyl betaine, an N-alkylaminopropionate, an N-alkyliminodipropionate, etc., can also be used.

In order to increase the dispersion stability, control the color hue of a dye formed from a polymer coupler latex dispersed and the oxidation product of an aromatic 50 primary amine developing agent and improve the bending property of the emulsion coated, a permanent solvent, that is, a water-immiscible organic solvent having a high boiling point (i.e., above 200° C.), may be added in a small amount (i.e., not more than 50% by weight 55 based on the polymer coupler). The concentration of the permanent solvent must be at such a low level that the copolymer is plasticized while it is maintained in solid particle form. Furthermore, it is desirable to use the permanent solvent in a relatively low concentration 60 in order to reduce the thickness of a final emulsion layer as much as possible to obtain good sharpness.

It is desirable if the ratio of the color forming portion in the polymer coupler latex is usually from 5 to 80% by weight. Particularly, a ratio from 20 to 70% by weight 65 is preferred in view of color reproducibility, color forming property and stability. In this case, an equivalent molecular weight, that is, a gram number of the

polymer containing 1 mol of a coupler monomer, is preferably from about 250 to 3,000, but it is not limited thereto.

The polymer coupler latex of the invention is used in a range of  $2 \times 10^{-3}$  to  $5 \times 10^{-1}$  mol, preferably  $1 \times 10^{-2}$  to  $5 \times 10^{-1}$  mol, of coupler unit per mol of silver.

Preferred specific examples of the coupler monomers used in the present invention are set forth below, but the present invention is not to be construed as being limited thereto.



-continued



-continued

(12)



10



(7)

15



20



(8)

25



30



(14)



(9) 35



40



(15)

(10)

45



50



55



(16)

(11)

60



65



(17)



11

-continued



12

-continued



The monomer coupler represented by the general formula (I) according to the present invention can be synthesized in the following reaction scheme:



-continued



### A. MONOMER COMPOUNDS

#### SYNTHESIS EXAMPLE 1

In the above formulae,  $\text{R}_1$ ,  $\text{R}_2$ ,  $\text{R}_3$ ,  $\text{X}$ ,  $\text{Y}$ ,  $\text{Z}$ ,  $\text{Ar}$ ,  $1$ ,  $m$  and  $n$  each has the same meaning as defined above,  $\text{X}'$  represents  $-\text{COCl}$ ,  $-\text{OCOCl}$  or  $-\text{N}=\text{C}=\text{O}$  and  $\text{X}''$  represents a halogen atom such as a chlorine atom, a bromine atom, etc.

Namely, the monomer coupler represented by the general formula (I) can be synthesized by reacting a compound represented by the general formula (IV) with a 3-amino-2-pyrazolin-5-one represented by the general formula (V) or through an intermediate product represented by the general formula (VI). Also, the monomer coupler can be synthesized through an intermediate product represented by the general formula (VIII) or (IX) which is obtained by reacting a compound represented by the general formula (VII) with a compound represented by the general formula (V).

The 3-amino-2-pyrazolin-5-one compound represented by the general formula (V) used can be synthesized by a ring-forming reaction of an appropriate aromatic hydrazine with  $\beta$ -amino- $\beta$ -ethoxypropionic acid as described in U.S. Pat. No. 2,376,380, British Pat. Nos. 1,069,533, 1,166,035, 1,190,914 and 1,269,355, or by a reaction of an aromatic hydrazine with an ester of  $\beta$ -ethoxy- $\beta$ -imino propionic acid as described in *J. Amer. Chem. Soc.*, Vol. 66, pages 1851 to 1855 (1944).

Typical synthesis examples of the monomer compounds and the polymer compounds used in the present invention are set forth below.

40

168 g (4.0 mol) of sodium hydroxide and 262 g (2.0 mol) of  $\epsilon$ -amino-n-caproic acid were dissolved in 400 ml of water and to the solution was added dropwise 181 g (2.0 mol) of acrylic chloride over a period of about 3 hours under cooling (at  $-20^\circ \text{C}$ .). To the mixture there was gradually added 200 ml of concentrated hydrochloric acid (36%) to acidify. After adding 1 liter of acetonitrile and 500 ml of water, the organic layer was separated and concentrated to half of its original volume under a reduced pressure by removing the solvent. To the residue was added 2 liters of chloroform, the mixture was washed with water and the chloroform was distilled off under a reduced pressure. The crystals deposited by cooling the residue were collected by filtration to obtain 215 g (58% yield) of 6-acryloylamino-n-caproic acid.

37.0 g (0.2 mol) of 6-acryloylamino-n-caproic acid thus obtained and 1.0 ml of nitrobenzene were dissolved in 250 ml of acetonitrile and to the solution was added 2.5 ml of dimethylformamide. To the mixture was added 16 ml (0.22 mol) of thionyl chloride under cooling (at  $10^\circ \text{C}$ .). After 2 hours, a nitrogen gas was bubbled and a hydrogen chloride gas was distilled off. The solution was added to 200 ml of acetonitrile containing 24.4 g (0.1 mol) of 3-amino-1-(2,5-

dichlorophenyl)-2-pyrazolin-5-one and 32.5 ml (0.4 mol) of pyridine dissolved under cooling (at 10° C.) with stirring. After being reacted for 1 hour, 200 ml of ethyl acetate was added, the mixture was washed 3 times with water and dried with anhydrous sodium sulfate. The ethyl acetate was distilled off under a reduced pressure, the crystals thus deposited were collected by filtration to obtain 26.0 g (45% yield) of 1-(2,5-dichlorophenyl)-3-(6'-acryloylaminohexanoylamino)-5-(6'-acryloylaminohexanoyloxy)-pyrazole.

26.0 g (0.045 mol) of the pyrazole derivative thus obtained was dissolved in 150 ml of methanol and to the solution was added 1.0 ml of nitrobenzene. To the mixture was added 150 ml of a methanol solution containing 2.8 g (0.05 mol) of potassium hydroxide under cooling (at 10° C.) with stirring. After about 15 minutes, the mixture was neutralized with glacial acetic acid, and the crystals thus deposited were collected by filtration and recrystallized from acetonitrile to obtain 12.9 g (70% yield) of Monomer Coupler (6).

Melting Point: 143° to 145° C.

Elemental Analysis for  $C_{18}H_{20}N_4O_3Cl_2$ : Calculated: C: 52.60%, H: 4.91%, N: 13.63%. Found: C: 52.72%, H: 5.03%, N: 13.86%.

### SYNTHESIS EXAMPLE 2

#### Synthesis of

1-(2,5-dichlorophenyl)-3-(2'-methacryloylaminoacetyl amino)-2-pyrazolin-5-one  
[Monomer Coupler (9)]

To 400 ml of water containing 80 g (2.0 mol) of sodium hydroxide dissolved, were added 150 g (2.0 mol) of glycine and 4 ml of nitrobenzene. To the mixture, there were simultaneously added 200 ml of an aqueous solution containing 96 g (2.4 mol) of sodium hydroxide and 230 g (2.2 mol) of methacrylic chloride under cooling (at -20° C.) with stirring over a period of about 2 hours. After adding 800 ml of acetonitrile and 160 ml of concentrated hydrochloric acid, the organic layer was separated. The solvent was distilled off under a reduced pressure and the crystals thus deposited were collected by filtration and recrystallized from ethyl acetate to obtain 184 g (64.3% yield) of  $\alpha$ -methacryloylaminoacetic acid.

72 g (0.5 mol) of  $\alpha$ -methacryloylaminoacetic acid thus obtained, 49 g (0.2 mol) of 3-amino-1-(2,5-dichlorophenyl)-2-pyrazolin-5-one, 2 ml of nitrobenzene and 110 ml (0.4 mol) of pyridine were dissolved in 750 ml of acetonitrile and to the mixture was added 33 ml (0.45 mol) of thionyl chloride under cooling (at 10° C.) with stirring. About about 2.5 hours, 250 ml of water was added to the reaction mixture and the crystals thus deposited were collected by filtration and recrystallized from acetonitrile to obtain 40 g (54.4% yield) of Monomer Coupler (9).

Melting Point: 232° to 235° C.

Elemental Analysis for  $C_{15}H_{14}N_4O_3Cl_2$ : Calculated: C: 48.82%, H: 3.82%, N: 15.18%. Found: C: 49.03%, H: 3.97%, N: 15.33%.

### SYNTHESIS EXAMPLE 3

#### Synthesis of

1-(2,4,6-trichlorophenyl)-3-[3'-(4"-vinylbenzene)sulfonylpropionylamino]-2-pyrazolin-5-one [Monomer Coupler (16)]

155 g (0.75 mol) of potassium 4-vinylbenzenesulfinate and 54 g (0.75 mol) of acrylic acid were dissolved in 500

ml of water and the solution was stirred at about 25° C. The crystals gradually deposited were collected by filtration and washed with water to obtain 65.5 g (36% yield) of  $\beta$ -(4-vinylbenzene)sulfonylpropionic acid.

32 g (0.133 mol) of  $\beta$ -(4-vinylbenzene)sulfonylpropionic acid thus obtained and 6 ml of nitrobenzene were dissolved in 400 ml of acetonitrile and to the solution was added 6 ml of dimethylformamide. To the mixture, there was added 15.8 g (0.16 mol) of thionyl chloride under cooling (at 10° C.) with stirring. After 2 hours, a nitrogen gas was bubbled and a hydrogen chloride gas was distilled off. The solution was added to 400 ml of tetrahydrofuran containing 18.5 g (0.067 mol) of 3-amino-1-(2,4,6-trichlorophenyl)-2-pyrazolin-5-one and 20 ml of pyridine dissolved. After being reacted for 1 hour, 300 ml of ethyl acetate was added to the reaction mixture, the mixture was washed twice with a saturated aqueous sodium chloride solution and dried with anhydrous sodium sulfate. The solvent was distilled off under a reduced pressure. The residual oily product was dissolved in 300 ml of ethanol and 200 ml of water, to which was added 25 ml of aqueous ammonia, and the mixture was stirred for about 30 minutes and neutralized with glacial acetic acid. Water was added to the mixture and the crystals thus deposited were collected by filtration and recrystallized from acetonitrile to obtain 26 g (78.2% yield) of Monomer Coupler (16).

Melting Point: above 250° C.

Elemental Analysis for  $C_{20}H_{16}N_3O_4SCl_3$ : Calculated: C: 47.96%, H: 3.22%, N: 8.39%. Found: C: 48.00%, H: 3.28%, N: 8.45%.

## B. POLYMER COMPOUNDS

#### Synthesis Method I

### SYNTHESIS EXAMPLE 4

Copolymer latex of  
1-(2,5-dichlorophenyl)-3-(2'-methacryloylaminoacetyl amino)-2-pyrazolin-5-one  
[Monomer Coupler (9)] and n-octyl methacrylate  
[Polymer Coupler Latex (A)]

2 liters of an aqueous solution containing 2 g of sodium salt of oleyl methyl tauride dissolved was stirred and heated to 95° C. while introducing nitrogen gas through the solution. To the mixture was added 40 ml of an aqueous solution containing 280 mg of potassium persulfate dissolved. 20 g of n-octyl methacrylate and 20 g of Monomer Coupler (9) were dissolved by heating in 400 ml of ethanol and the resulting solution was added to the above-described aqueous solution at an interval of about 30 minutes while preventing the deposition of crystals. After the completion of the addition, the mixture was heated at from 85° C. to 95° C. with stirring for 45 minutes, to which was then added 40 ml of an aqueous solution containing 120 mg of potassium persulfate dissolved. After being reacted for 1 hour, the n-octyl methacrylate not reacted were distilled off as an azeotropic mixture with water. The latex thus-formed was cooled, pH of which was adjusted to 6.0 with a 1N sodium hydroxide solution and filtered. The concentration of the polymer in the latex was 10.15% and it was found that the copolymer synthesized contained 48.5% of Monomer Coupler (9) as the result of nitrogen analysis.

## SYNTHESIS EXAMPLE 5

## Copolymer latex of

1-(2,5-dichlorophenyl)-3-(6'-acryloylaminohex-  
anoylamino)-2-pyrazolin-5-one [Monomer Coupler (6)]  
and n-butyl acrylate [Polymer Coupler Latex (B)]

2 liters of an aqueous solution containing 2 g of sodium salt of oleyl methyl tauride dissolved was stirred and heated to 95° C. while introducing nitrogen gas through the solution. To the mixture was added 40 ml of an aqueous solution containing 280 mg of potassium persulfate dissolved. 30 g of n-butyl acrylate and 10 g of Monomer Coupler (6) were dissolved by heating in 400 ml of ethanol and the resulting solution was added to the above-described aqueous solution at an interval of about 30 minutes while preventing the deposition of crystals. After the completion of the addition, the mixture was heated at from 85° C. to 95° C. with stirring for 45 minutes, to which was then added 40 ml of an aqueous solution containing 120 mg of potassium persulfate dissolved. After being reacted for 1 hour, the n-butyl acrylate not reacted were distilled off as an azeotropic mixture with water. The latex thus-formed was cooled, pH of which was adjusted to 6.0 with a 1N sodium hydroxide solution and filtered. The concentration of the polymer in the latex was 10.52% and it was found that copolymer synthesized contained 23.7% of Monomer Coupler (6) as the result of nitrogen analysis.

## SYNTHESIS EXAMPLE 6

## Copolymer latex of

1-(2,4-dichlorophenyl)-3-(2'-acryloylamino-  
propionylamino)-2-pyrazolin-5-one [Monomer Coupler (22)] and ethyl acrylate [Polymer Coupler Latex (C)]

270 ml of an aqueous solution containing 1.54 g of sodium salt of oleyl methyl tauride dissolved was stirred and heated to 95° C. while introducing nitrogen gas through the solution. To the mixture were added 20 ml of an aqueous solution containing 28 mg of potassium persulfate dissolved, and then 2.8 g of ethyl acrylate. The mixture was polymerized by heating at from 85° C. to 90° C. with stirring for about 1 hour to prepare Latex (a). Then, to Latex (a) were added 14 g of Monomer Coupler (22), 100 ml of ethanol and 10 ml of an ethanol solution containing 14 g of ethyl acrylate dissolved. To the mixture was then added 50 ml of an aqueous solution containing 196 mg of potassium persulfate dissolved and the mixture was polymerized by heating with stirring. After being reacting for 1 hour, 30 ml of an aqueous solution containing 84 mg of potassium persulfate was further added to the mixture and the mixture was continuously reacted for 1.5 hours. The ethanol and the ethyl acrylate not reacted were distilled off as an azeotropic mixture with water. The latex thus-formed was cooled, pH of which was adjusted to 6.0 with a 1N sodium hydroxide solution and filtered. The concentration of the polymer in the latex was 10.3% and it was found that the copolymer synthesized contained 45.7% of Monomer Coupler (22) as the result of nitrogen analysis.

## Synthesis Method II

## Synthesis Example 7

Synthesis of Copolymer coupler of  
1-(2,4,6-trichlorophenyl)-3-[3'-(4"-vinylbenzene)sulfonylpropionylamino]-2-pyrazolin-5-one [Monomer Coupler (16)] and methyl acrylate [Oleophilic Polymer Coupler (I)]

10 20 g of Monomer Coupler (16) and 20 g of methyl acrylate were added to 150 ml of dioxane and dissolved by heating at 85° C. To the solution was added 350 mg of 2,2'-azobis(2,4-dimethylvaleronitrile) dissolved in 100 ml of dioxane, the mixture was heated for about 3 hours and further heated at 90° C. for 2 hours. The resulting solution was then poured into 2 liters of ice water and the solid thus deposited was collected by filtration and thoroughly washed with water. By drying the product under a reduced pressure with heating, 38.5 g of Oleophilic Polymer Coupler (I) was obtained. It was found that the oleophilic polymer coupler contained 53.2% of Monomer Coupler (16) in the copolymer synthesized as the result of nitrogen analysis.

A method for dispersing Oleophilic Polymer Coupler (I) in an aqueous gelatin solution in a form of latex is described in the following.

## Synthesis of Polymer Coupler Latex (I')

Two solutions (a) and (b) were prepared in the following manner.

Solution (a): 300 g of a 5% by weight aqueous solution of bone gelatin (pH of 5.6 at 35° C.) was heated to 32° C. and to which was added 12 ml of a 10% by weight aqueous solution of sodium lauryl sulfate.

Solution (b): 20 g of the oleophilic polymer coupler described above was dissolved in 60 g of ethyl acetate at 38° C.

Solution (b) was put into a mixer with explosion preventing equipment while stirring at a high speed to which was rapidly added solution (a). After stirring for 1 minute, the mixer was stopped and ethyl acetate was removed by distillation under a reduced pressure. Thus, the oleophilic polymer coupler was dispersed in a diluted gelatin solution to prepare Polymer Coupler Latex (I').

## Synthesis Example 8

Synthesis of Copolymer coupler of  
1-(2,5-dichlorophenyl)-3-(2'-methacryloylaminoacetylaminoo)-2-pyrazolin-5-one  
[Monomer Coupler (9)] and methyl acrylate [Oleophilic Polymer Coupler (II)]

20 g of Monomer Coupler (9) and 20 g of methyl acrylate were added to 150 ml of tertiary butanol and the mixture was refluxed by heating with stirring. To the mixture was added 350 mg of azobisisobutyronitrile dissolved in 10 ml of tertiary butanol and the mixture was refluxed by heating for about 3 hours. The resulting solution was then poured into 2 liters of ice water and the solid thus deposited was collected by filtration and thoroughly washed with water. The solid was dissolved in ethyl acetate and reprecipitated with n-hexane. By drying the product under a reduced pressure with heating, 37.9 g of Oleophilic Polymer Coupler (II) was obtained. It was found that the oleophilic polymer coupler contained 52.7% of Monomer Coupler (9) in the copolymer synthesized as the result of nitrogen analysis.

## Synthesis of Polymer Coupler Latex (II')

Two solutions (a) and (b) were prepared in the following manner.

Solution (a): 200 g of a 3.0% by weight aqueous solution of bone gelatin (pH of 5.6 at 35° C.) was heated to 38° C. and to which was added 16 ml of a 10% by weight aqueous solution of sodium lauryl sulfate.

Solution (b): 20 g of Oleophilic Polymer Coupler (II)

luted gelatin solution to prepare Polymer Coupler Latex (II').

## SYNTHESIS EXAMPLES 9 TO 25

Using the above-described monomer couplers, the magenta polymer coupler latexes described below were prepared in the same manner as described for the copolymers in Synthesis Examples 4 to 6 (Synthesis Method I).

| Synthesis Example | Polymer Coupler Latexes by Synthesis Method I |                 |            |                |            |      | Monomer Coupler Unit in Polymer (wt %) |
|-------------------|-----------------------------------------------|-----------------|------------|----------------|------------|------|----------------------------------------|
|                   | Polymer Coupler Latex                         | Monomer Coupler | Amount (g) | (*1) Comonomer | Amount (g) |      |                                        |
| 9                 | (D)                                           | (1)             | 20         | MA             | 20         | 54.2 |                                        |
| 10                | (E)                                           | (3)             | 10         | BA             | 40         | 19.7 |                                        |
| 11                | (F)                                           | (3)             | 10         | EA             | 40         | 21.3 |                                        |
| 12                | (G)                                           | (6)             | 10         | BA             | 20         | 33.5 |                                        |
| 13                | (H)                                           | (8)             | 20         | EA             | 20         | 51.6 |                                        |
| 14                | (I)                                           | (9)             | 20         | MMA            | 20         | 50.7 |                                        |
| 15                | (J)                                           | (9)             | 20         | OA             | 20         | 49.1 |                                        |
| 16                | (K)                                           | (9)             | 20         | OMA            | 30         | 40.7 |                                        |
| 17                | (L)                                           | (9)             | 20         | MA/BA          | 10/10      | 50.3 |                                        |
| 18                | (M)                                           | (9)             | 10         | EA             | 40         | 20.4 |                                        |
| 19                | (N)                                           | (10)            | 20         | MA             | 20         | 53.2 |                                        |
| 20                | (O)                                           | (14)            | 20         | BA             | 20         | 50.2 |                                        |
| 21                | (P)                                           | (15)            | 30         | MA             | 20         | 61.7 |                                        |
| 22                | (Q)                                           | (16)            | 10         | BA             | 20         | 33.8 |                                        |
| 23                | (R)                                           | (17)            | 20         | OMA            | 20         | 49.5 |                                        |
| 24                | (S)                                           | (25)            | 10         | BA             | 40         | 20.5 |                                        |
| 25                | (T)                                           | (25)            | 10         | EA             | 40         | 19.6 |                                        |

(\*1) MA: Methyl Acrylate

MMA: Methyl Methacrylate

EA: Ethyl Acrylate

BA: n-Butyl Acrylate

OA: n-Octyl Acrylate

OMA: n-Octyl Methacrylate

described above was dissolved in 200 ml of ethyl acetate at 38° C.

Solution (b) was put into a mixer with explosion preventing equipment while stirring at high speed and to which was rapidly added Solution (a). After stirring for 1 minute, the mixer was stopped and ethyl acetate was removed by distillation under a reduced pressure. Thus, the oleophilic polymer coupler was dispersed in a di-

The amounts of the monomer couplers and the comonomers in the above table indicate amounts used in the synthesis of the polymer coupler latexes.

## SYNTHESIS EXAMPLES 26 TO 43

Using the above-described monomer couplers, the oleophilic magenta polymer couplers described below were prepared in the same manner as described for the copolymers in Synthesis Examples 7 and 8 (Synthesis Method II).

| Synthesis Example | Oleophilic Polymer Coupler by Synthesis Method II |                 |            |                |            |      | Monomer Coupler Unit in Polymer (wt %) |
|-------------------|---------------------------------------------------|-----------------|------------|----------------|------------|------|----------------------------------------|
|                   | Oleophilic Polymer Coupler                        | Monomer Coupler | Amount (g) | (*1) Comonomer | Amount (g) |      |                                        |
| 26                | (III)                                             | (3)             | 20         | MA             | 20         | 52.1 |                                        |
| 27                | (IV)                                              | (3)             | 10         | BA             | 40         | 20.5 |                                        |
| 28                | (V)                                               | (8)             | 20         | MA             | 20         | 50.9 |                                        |
| 29                | (VI)                                              | (9)             | 20         | MA             | 20         | 51.2 |                                        |
| 30                | (VII)                                             | (9)             | 30         | BA             | 20         | 58.7 |                                        |
| 31                | (VIII)                                            | (9)             | 20         | EHA            | 30         | 40.9 |                                        |
| 32                | (IX)                                              | (11)            | 20         | MA             | 10         | 69.3 |                                        |
| 33                | (X)                                               | (12)            | 20         | MA/EA          | 10/10      | 50.6 |                                        |
| 34                | (XI)                                              | (15)            | 20         | PA             | 20         | 49.8 |                                        |
| 35                | (XII)                                             | (16)            | 20         | MA             | 20         | 50.9 |                                        |
| 36                | (XIII)                                            | (16)            | 20         | BMA            | 20         | 47.8 |                                        |
| 37                | (XIV)                                             | (17)            | 20         | MA             | 20         | 48.7 |                                        |
| 38                | (XV)                                              | (17)            | 20         | BA             | 20         | 50.3 |                                        |
| 39                | (XVI)                                             | (18)            | 10         | BA             | 20         | 31.5 |                                        |
| 40                | (XVII)                                            | (20)            | 20         | MA             | 20         | 51.3 |                                        |
| 41                | (XVIII)                                           | (22)            | 20         | MA             | 20         | 53.7 |                                        |
| 42                | (XIX)                                             | (24)            | 20         | BA             | 20         | 50.1 |                                        |

-continued

## Oleophilic Polymer Coupler by Synthesis Method II

| Synthesis Example | Oleophilic Coupler | Monomer Coupler | Amount (g) | (*)1 Comonomer | Amount (g) | Monomer Coupler Unit in Polymer (wt %) |
|-------------------|--------------------|-----------------|------------|----------------|------------|----------------------------------------|
| 43                | (XX)               | (25)            | 20         | BA             | 20         | 49.3                                   |

(\*1) MA: Methyl Acrylate  
 EA: Ethyl Acrylate  
 PA: n-Propyl Acrylate  
 BA: n-Butyl Acrylate  
 BMA: n-Butyl Methacrylate  
 EHA: 2-Ethylhexyl Acrylate

The amounts of the monomer couplers and the comonomers in the above table indicate amounts used in the 15 synthesis of the polymer coupler latexes.

Dispersion of these oleophilic polymer couplers can be carried out in the same manner as described in Synthesis Examples 7 and 8 and specific methods are described in the examples hereinafter.

The 4-equivalent magenta polymer coupler latexes according to the present invention can be used individually or as mixtures of two or more thereof.

The 4-equivalent magenta polymer coupler latexes according to the present invention can also be used 25 together with a 4-equivalent magenta polymer coupler latex, such as those described in U.S. Pat. No. 4,080,211, British Pat. No. 1,247,688, etc.

Further, a dispersion which is prepared by dispersing a hydrophobic magenta color forming coupler, for example, a magenta coupler, as described in U.S. Pat. Nos. 2,600,788, 2,983,608, 3,062,653, 3,127,269, 3,311,476, 3,419,391, 3,519,429, 3,558,319, 3,582,322, 3,615,506, 3,834,908 and 3,891,445, West German Pat. No. 1,810,464, West German Patent Application (OLS) 35 Nos. 2,408,665, 2,417,945, 2,418,959 and 2,424,467, Japanese Patent Publication No. 6031/65, Japanese Patent Application (OPI) Nos. 20826/76, 58922/77, 129538/74, 74027/74, 159336/75, 42121/77, 74028/74, 60233/75, 26541/76 and 55122/78 (the term "OPI" as used herein refers to a "published unexamined Japanese patent application"), etc., in a hydrophilic colloid in a manner as described, for example, in U.S. Pat. Nos. 2,269,158, 2,272,191, 2,304,940, 2,311,020, 2,322,027, 2,360,289, 2,772,163, 2,801,170, 2,801,171 and 3,619,195, British Pat. No. 1,151,590, West German Pat. No. 1,143,707, etc., is loaded into the 4-equivalent magenta polymer coupler latex according to the present invention in a manner as described in Japanese Patent Application (OPI) No. 39853/76, etc., and the resulting latex can be used. It is also possible for the above-described hydrophobic magenta coupler to be loaded into the 4-equivalent magenta polymer coupler latex according to the present invention in a manner as described in Japanese Patent Application (OPI) Nos. 59942/76 and 32552/79, U.S. Pat. No. 4,199,363, etc., and the resulting latex can be used. The term "load" used herein refers to the state in which a hydrophobic magenta coupler is incorporated into the interior of a 4-equivalent magenta polymer coupler latex, or a state in which 60 a hydrophobic magenta coupler is deposited on the surface of a 4-equivalent magenta polymer coupler latex. However, the mechanism by which the load occurs is not accurately known.

In order to satisfy the characteristics required of the photographic light-sensitive material, a dispersion which is prepared by dispersing a development inhibitor releasing (DIR) coupler as described, for example,

in U.S. Pat. Nos. 3,148,062, 3,227,554, 3,733,201, 3,617,291, 3,703,375, 3,615,506, 3,265,506, 3,620,745, 3,632,345, 3,869,291, 3,642,485, 3,770,436 and 3,808,945, British Pat. Nos. 1,201,110 and 1,236,767, etc., in a hydrophilic colloid in a manner as described in U.S. Pat. Nos. 2,269,158, 2,272,191, 2,304,940, 2,311,020, 2,322,027, 2,360,289, 2,772,163, 2,801,170, 2,801,171 and 3,619,195, British Pat. No. 1,151,590, West German Pat. No. 1,143,707, etc., is loaded into the 4-equivalent magenta polymer coupler latex according to the present invention in a manner as described in Japanese Patent Application (OPI) No. 39853/76. The resulting latex can then be used, or the above-described DIR coupler is loaded into the 4-equivalent magenta polymer coupler latex in a manner as described in Japanese Patent Application (OPI) Nos. 59942/76 and 32552/79, U.S. Pat. No. 4,199,363, etc., and the resulting latex can then be used.

Furthermore, the 4-equivalent magenta polymer coupler latex according to the present invention can be used together with a DIR compound as described, for example, in West German Patent Application (OLS) Nos. 2,529,350, 2,448,063 and 2,610,546, U.S. Pat. Nos. 3,928,041, 3,958,993, 3,961,959, 4,049,455, 4,052,213, 3,379,529, 3,043,690, 3,364,022, 3,297,445 and 3,287,129.

Moreover, the 4-equivalent magenta polymer coupler latex according to the present invention can be used in combination with a colored magenta coupler as described, for example, in U.S. Pat. No. 2,449,966, West German Pat. No. 2,024,186, Japanese Patent Application (OPI) Nos. 123625/74, 131448/74 and 42121/77, etc., a competing coupler as described, for example, in U.S. Pat. Nos. 3,876,428, 3,580,722, 2,998,314, 2,808,329, 2,742,832 and 2,689,793, etc., a stain preventing agent as described, for example, in U.S. Pat. Nos. 2,336,327, 2,728,659, 2,336,327, 2,403,721, 2,701,197 and 3,700,453, etc., a dye image stabilizing agent as described, for example, in British Pat. No. 1,326,889, U.S. Pat. Nos. 3,432,300, 3,698,909, 3,574,627, 3,573,050 and 3,764,337, etc., or the like.

The color photographic light-sensitive material produced according to the present invention can also contain conventional coupler(s) other than a magenta color forming coupler. A non-diffusible coupler which contains a hydrophobic group, called a ballast group, in the molecule thereof is preferred as a coupler. A coupler can have either a 4-equivalent or a 2-equivalent property with respect to the silver ion. In addition, a colored coupler providing a color correction effect, or a coupler which releases a development inhibitor upon a development can also be present therein. Furthermore, a coupler which provides a colorless product upon coupling can be employed.

A known open chain ketomethylene type coupler can be used as a yellow color forming coupler. Of these couplers, benzoyl acetanilide type and pivaloyl acetanilide type compounds are especially effective. Specific examples of yellow color forming couplers which can be employed are described, for example, in U.S. Pat. Nos. 2,875,057, 3,265,506, 3,408,194, 3,551,155, 3,582,322, 3,725,072 and 3,891,445, West German Pat. No. 1,547,868, West German Patent Application (OLS) Nos. 2,219,917 2,261,361 and 2,414,006, British Pat. No. 1,425,020, Japanese Patent Publication No. 10783/76, Japanese Patent Application (OPI) Nos. 26133/72, 73147/73, 102636/76, 6341/75, 123342/75, 130442/75, 21827/76 and 87650/75, etc.

A phenol type compound, a naphthol type compound, etc., can be employed as a cyan color forming coupler. Specific examples of cyan color forming couplers which can be employed are those described, for example, in U.S. Pat. Nos. 2,369,929, 2,434,272, 2,474,293, 2,521,908, 2,895,826, 3,034,892, 3,311,476, 3,458,315, 3,476,563, 3,583,971, 3,591,383, 3,767,411 and 4,004,929, West German Patent Application (OLS) Nos. 2,414,830 and 2,454,329, Japanese Patent Application (OPI) Nos. 59838/73, 26034/76, 5055/73, 146828/76, 73050/80, etc.

Two or more kinds of the coupler described above can be incorporated into the same layer, or the same coupler compound can also be present in two or more layers.

A known method, for example, the method described in U.S. Pat. No. 2,322,027, can be used in order to incorporate the couplers described above into a silver halide emulsion layer. The coupler is dispersed in a hydrophilic colloid and then mixed with a silver halide emulsion. When a coupler having an acid group such as a carboxylic acid group, a sulfonic acid group, etc., is used, it can be incorporated into a hydrophilic colloid as an alkaline aqueous solution thereof.

The silver halide emulsions which can be used in the present invention are those wherein silver chloride, silver bromide, or a mixed silver halide such as silver chlorobromide, silver, iodobromide, or silver chloroiodobromide is finely dispersed in a hydrophilic polymer such as gelatin. The silver halide can be chosen depending on the intended use of the photographic light-sensitive material from dispersions having a uniform grain size or those having a wide grain size distribution or from dispersions having an average grain size of from about 0.1 micron to 3 microns. These silver halide emulsions can be prepared, for example, by a single jet method, by a double jet method or a controlled double jet method, or by a ripening method such as an ammonia method, a neutral method, or an acid method. Also, these silver halide emulsions can be subjected to chemical sensitization such as a sulfur sensitization, a gold sensitization, a reduction sensitization, etc., and can contain a speed increasing agent such as a polyoxyethylene compound, an onium compound, etc. Further, a silver halide emulsion of the type wherein latent images are predominantly formed on the surface of the grains or of the type where latent images are predominantly formed inside the grains can be used in the present invention. Also, two or more kinds of silver halide photographic emulsions prepared separately and then mixed can be employed.

As a hydrophilic high molecular weight substance composed of the photographic light-sensitive layer of the present invention, a protein such as gelatin, etc., a

high molecular weight non-electrolyte such as polyvinyl alcohol, polyvinyl pyrrolidone, polyacrylamide, etc., an acidic polymer such as an alginate, a polyacrylic acid salt, etc., a high molecular weight amphotile such as a polyacryamide treated by the Hoffman rearrangement reaction, a copolymer of acrylic acid and N-vinylimidazole, etc., a cross-linking polymer as described in U.S. Pat. No. 4,215,195, and the like are suitable. Furthermore, a hydrophobic polymer dispersion such as a latex of polybutyl acrylate, etc., can be included in the continuous phase of such a hydrophilic high molecular weight substance.

The silver halide emulsion used in the present invention can be chemically sensitized, as noted above, using conventional methods. Examples of suitable chemical sensitizers include, for example, gold compounds such as chloroaurates and gold trichloride as described in U.S. Pat. Nos. 2,399,083, 2,540,085, 2,597,856, and 2,597,915; salts of a noble metal, such as platinum, palladium, iridium, rhodium and ruthenium, as described in U.S. Pat. Nos. 2,448,060, 2,540,086, 2,566,245, 2,566,263 and 2,598,079; sulfur compounds capable of forming silver sulfide by reacting with a silver salt, such as those described in U.S. Pat. Nos. 1,574,944, 2,410,689, 3,189,458 and 3,501,313; stannous salts, amines, and other reducing compounds such as those described in U.S. Pat. Nos. 2,487,850, 2,518,698, 2,521,925, 2,521,926, 2,694,637, 2,983,610 and 3,201,254 and the like.

Various compounds can be added to the photographic emulsions used in the present invention in order to prevent a reduction of the sensitivity or a formation of fog during preparation, storage, or processing. A wide variety of such compounds are known, such as heterocyclic compounds, mercury-containing compounds, mercapto compounds or metal salts, including 4-hydroxy-6-methyl-1,2,3a,7-tetraazaindene, 3-methylbenzothiazole and 1-phenyl-5-mercaptopentetrazole. Other examples of such compounds which can be used are described, for example, in U.S. Pat. Nos. 1,758,576, 2,110,178, 2,131,038, 2,173,628, 2,697,040, 2,304,962, 2,324,123, 2,394,198, 2,444,605-8, 2,566,245, 2,694,716, 2,697,099, 2,708,162, 2,728,663-5, 2,476,536, 2,824,001, 2,843,491, 2,886,437, 3,052,544, 3,137,577, 3,220,839, 3,226,231, 3,236,652, 3,251,691, 3,252,799, 3,287,135, 3,326,681, 3,420,668 and 3,622,339, British Pat. Nos. 893,428; 403,789, 1,173,609 and 1,200,188, as well as in K. Mees, *The Theory of the Photographic Process*, 3rd Ed. (1966) and the literature references cited therein.

The photographic emulsion used in the present invention can also contain one or more surface active agents. These surface active agents are commonly used as a coating aid. However, in some cases they are used as an emulsifier, a dispersant, a sensitizer, an antistatic agent, or an adhesion preventing agent.

The surface active agents can be classified into various groups, as follows: natural surface active agents such as saponin; nonionic surface active agents such as alkylene oxides, glycerols and glycidols; cationic surface active agents such as higher alkylamines, quaternary ammonium salts, heterocyclic compounds such as pyridine and the like, phosphoniums or sulfoniums; anionic surface active agents containing an acid group such as a carboxylic acid group, a sulfonic acid group, a phosphoric acid group, a sulfuric acid ester group, or phosphoric acid ester group; amphoteric surface active agents such as aminoacids, aminosulfonic acids, aminoalcohol sulfuric acid esters or aminoalcohol phos-

phoric acid esters. Some examples of those surface active agents which can be used are described in U.S. Pat. Nos. 2,271,623, 2,240,472, 2,288,226, 2,739,891, 3,068,101, 3,158,484, 3,201,253, 3,210,191, 3,294,540, 3,415,649, 3,441,413, 3,442,654, 3,475,174, 3,545,974, West German Patent Application (OLS) No. 1,942,665, British Pat. Nos. 1,077,317, and 1,198,450, as well as Ryohei Oda et al., *Kaimenkasseizai no Gosei to Sono Oyo (Synthesis and Application of Surface Active Agents)*, Maki Shoten (1964), A. W. Perry, *Surface Active Agents*, Interscience Publications, Inc. (1958) and J. P. Sisley, *Encyclopedia of Surface Active Agents*, Vol. II, Chemical Publishing Co. (1964).

The photographic emulsions can be spectrally sensitized, or supersensitized, using a cyanine-type dye, such as a cyanine, merocyanine, carbocyanine, etc., individually, in combinations, or in combination with a styryl dye.

These spectral sensitization techniques are well known, and are described, for example, in U.S. Pat. Nos. 2,688,545, 2,912,329, 3,397,060, 3,615,635 and 3,628,964, British Pat. Nos. 1,195,302, 1,242,588 and 1,293,862, West German Patent Application (OLS) Nos. 2,030,326 and 2,121,780, Japanese Patent Publication Nos. 4936/68 and 14030/69, etc. The sensitizers can be selected as desired depending on the purposes and use of the photographic materials to be sensitized.

The hydrophilic colloid layer, and in particular a gelatin layer in the photographic light-sensitive material used in the present invention, can be hardened using various kinds of cross-linking agents. For instance, an inorganic compound such as a chromium salt and a zirconium salt, or an aldehyde type cross-linking agent such as mucochloric acid, or 2-phenoxy-3-chloromalealdehydic acid as described in Japanese Patent Publication No. 1872/71 can be effectively used in the present invention. However, non-aldehyde type cross-linking agents such as compounds having plural epoxy rings as described in Japanese Patent Publication No. 7133/59, the poly(1-aziridinyl) compounds as described in Japanese Patent Publication No. 8790/62, the active halogen compounds as described in U.S. Pat. Nos. 3,362,827 and 3,325,287 and the vinyl sulfone compounds as described in U.S. Pat. Nos. 2,994,611 and 3,582,322, Belgian Pat. No. 686,440, etc., are particularly suitable for use in the photographic light-sensitive material of the present invention.

The silver halide photographic emulsion of the present invention is suitably applied to a support. Illustrative supports include rigid materials such as glass, metal and ceramics, and flexible materials and the type of support chosen depends on the end-use objects. Typical examples of flexible supports include a cellulose nitrate film, a cellulose acetate film, a polyvinyl acetal film, a polystyrene film, a polyethylene terephthalate film, a polycarbonate film and a laminate thereof, a baryta coated paper, a paper coated with an  $\alpha$ -olefin polymer, such as polyethylene, polypropylene and an ethylene-butene copolymer, a plastic film having a roughened surface as described in Japanese Patent Publication No. 19068/72, and the like. Depending upon the end-use objects of the photographic light-sensitive material, the support can be transparent, colored by adding a dye or pigment, opaque by adding, for example, titanium white, or light-shielding by adding, for example, carbon black.

The layer of the photographic light-sensitive material can be coated on a support using various coating meth-

ods, including a dip coating method, an air-knife coating method, a curtain coating method, an extrusion coating method using a hopper as described in U.S. Pat. No. 2,681,294. Also, two or more layers can be coated simultaneously, using methods as described in U.S. Pat. Nos. 2,761,791, 3,508,947, 2,941,898, 3,526,528, etc.

The present invention is applicable to not only the so-called multilayer type photographic light-sensitive material comprising a support having superimposed thereon emulsion layers, each of which is sensitive to radiation of a substantially different wavelength region and forms color images of a substantially different hue, but also the so-called mixed packet type photographic light-sensitive material comprising a support having coated thereon a layer containing packets which are sensitive to radiation of substantially different wavelength regions and form color images of a substantially different hue. The present invention can be applied to a color negative film, a color positive film, a color reversal film, a color printing paper, a color reversal printing paper, and the like.

The color photographic light-sensitive material of the present invention is, after exposure, subjected to a development processing to form dye images. Development processing includes basically a color development step, a bleaching step and a fixing step. Each step can be carried out individually or two or more steps can be combined as one step where a processing solution having two or more functions is used. Also, each step can be separated into two or more steps. The development processing can further include a pre-hardening step, a neutralization step, a first development (black-and-white development) step, a stabilizing step, a water washing step, and the like, if desired. The temperature of processing can be varied depending on the photographic light-sensitive material, the processing method, and the like. In general, the processing steps are carried out at a temperature from 18° C. to 60° C. These steps need not necessarily be conducted at the same temperature.

A color developer solution is an alkaline solution having a pH of more than 8, preferably from 9 to 12, and containing, as a developing agent, a compound whose oxidation product is capable of forming a colored compound when reacted with a color forming agent, i.e., a color coupler. The developing agent described above includes a compound capable of developing an exposed silver halide and having a primary amino group on an aromatic ring, and a precursor which forms such compound. Typical examples of preferred developing agents are, for example, 4-amino-N,N-diethylaniline, 3-methyl-4-amino-N,N-diethylaniline, 4-amino-N-ethyl-N- $\beta$ -hydroxyethylaniline, 3-methyl-4-amino-N-ethyl-N- $\beta$ -hydroxyethylaniline, 4-amino-3-methyl-N-ethyl-N- $\beta$ -methanesulfonamidoethylaniline, 4-amino-N,N-dimethylaniline, 4-amino-3-methoxy-N,N-diethylaniline, 4-amino-3-methyl-N-ethyl-N- $\beta$ -ethoxyethylaniline, 4-amino-3-methoxy-N-ethyl-N- $\beta$ -methoxyethylaniline, 4-amino-3- $\beta$ -methanesulfonamidoethyl-N,N-diethylaniline, and the salts thereof (for example, the sulfates, the hydrochlorides, the sulfites, the p-toluenesulfonates, and the like). Other developing agents such as those described in U.S. Pat. Nos. 2,193,015 and 2,592,364, Japanese Patent Application (OPI) No. 64933/73, L. F. A. Mason, *Photographic Processing Chemistry*, pages 226-229; Focal Press, London (1966), T. H. James, *The Theory of the Photographic Process*, 4th Edition, pages 315-320, Macmillan, New York (1977),

etc., can be used. Further, an aminophenol as described in T. H. James, *The Theory of the Photographic Process*, 4th Edition, pages 311-315, etc., can be used. Also, a 3-pyrazolidone developing agent can be used together with these developing agents.

The color developer solution can optionally contain various additives. Typical examples of such additives include alkaline agents (for example, alkali metal or ammonium hydroxides, carbonates or phosphates); pH-adjusting agents or buffers (for example, weak acids such as acetic acid, boric acid, etc., weak bases, or salts thereof); developing accelerators (for example, various pyridinium compounds or cationic compounds such as those described in U.S. Pat. Nos. 2,648,604 and 3,671,247; potassium nitrate; sodium nitrate; condensation products of polyethylene glycol, and their derivatives such as those described in U.S. Pat. Nos. 2,533,990, 2,577,127 and 2,950,970; nonionic compounds such as polythioethers represented by those described in British Pat. Nos. 1,020,033 and 1,020,032; polymeric compounds having sulfite ester groups such as those described in U.S. Pat. No. 3,068,097; organic amines such as pyridine and ethanolamine; benzyl alcohol; hydrazines and the like); anti-fogging agents (for example, alkali metal bromides; alkali metal iodides; nitrobenzimidazoles such as those described in U.S. Pat. Nos. 2,496,940 and 2,656,271; mercaptobenzimidazole; 5-methylbenztriazole; 1-phenyl-5-mercaptopotetrazole; compounds for use in rapid processing such as those described in U.S. Pat. Nos. 3,113,864, 3,342,596, 3,295,976, 3,615,522 and 3,597,199; thiosulfonyl compounds such as those described in British Pat. No. 972,211; phenazine-N-oxides such as those described in Japanese Patent Publication No. 41675/71; those described in *Kagaku Shashin Binran (Manual of Scientific Photography)*, Vol. II, pages 29-47, and the like); stain or sludge preventing agents such as those described in U.S. Pat. Nos. 3,161,513 and 3,161,514, and British Pat. Nos. 1,030,442, 1,144,481 and 1,251,558; interlayer-effect accelerators disclosed in U.S. Pat. No. 3,536,487; preservatives (for example, sulfites, bisulfites, hydroxyamine hydrochloride, formsulfite, alkanolaminesulfite adducts, etc.) and the like.

The color photographic light-sensitive material of the present invention can be treated with various solutions prior to color development.

In the case of color reversal films, treatment with a first development solution is also carried out prior to the color development. As the first development solution, an alkaline aqueous solution containing at least one developing agent, such as hydroquinone, 1-phenyl-3-pyrazolidone, N-methyl-p-aminophenol and the like can be employed. The solution can also contain inorganic salts such as sodium sulfate; pH-adjusting agents or buffers such as borax, boric acid, sodium hydroxide and sodium carbonate; development fog inhibitors such as alkali metal halides (such as potassium bromide, etc.), and the like.

The additives illustrated above and the amounts thereof employed are well known in the color processing field.

After color development, the color photographic materials are usually bleached and fixed. The processes can be effected in a blix bath which combines the bleaching and fixing steps. Various compounds can be used as a bleaching agent, for example, ferricyanides; dichromates; water-soluble iron (III) salts; water-soluble cobalt (III) salts; water-soluble copper (II) salts;

water-soluble quinones; nitrosophenols; complex salts of a polyvalent cation such as iron (III), cobalt (III), copper (II), etc., and an organic acid, for example, metal complex of an aminopolycarboxylic acid such as ethylenediaminetetraacetic acid, nitrilotriacetic acid, iminodiacetic acid, N-hydroxyethylethylenediaminetriacetic acid, etc., malonic acid, tartaric acid, malic acid, diglycolic acid and dithioglycolic acid, and copper complex salt of 2,6-dipicolinic acid; peracids such as alkylperacids, persulfates, permanganates and hydrogen peroxide; hypochlorites; chlorine; bromine; bleaching powder; and the like. These can be suitably used, individually or in combination. To the bleaching solution, bleaching accelerators such as those described in U.S. Pat. Nos. 3,042,520 and 3,241,966, Japanese Patent Publication Nos. 8506/70 and 8836/70 and various other additives can be added.

Any known fixing solution can be used for fixing the photographic materials of the present invention. That is, ammonium, sodium, or potassium thiosulfate can be used as a fixing agent at a concentration of about 50 to about 200 g/liter. Fixing solutions can further contain stabilizers such as sulfites and metabisulfites; hardeners such as potassium alum; pH buffers such as acetates and borates, and the like. The fixing solution generally has a pH of more than 3 or less.

Bleaching baths, fixing baths and blixing baths as described, for example, in U.S. Pat. No. 3,582,322, Japanese Patent Application (OPI) No. 101934/73, West German Pat. No. 1,051,117 can also be employed.

The present invention will be explained in greater detail with reference to the following examples, but the present invention should not be construed as being limited thereto.

#### EXAMPLE 1

20 g of each of Oleophilic Polymer Couplers (I), (II), (XVII), (III) and (VII) according to the present invention and Comparative Oleophilic Polymer Couplers (a), (b), (c) and (d) was dissolved by heating in 60 ml of ethyl acetate and the solution was added to 300 ml of an aqueous solution containing 15 g of gelatin and 1.2 g of sodium lauryl sulfate. The resulting mixture was dispersed using a colloid mill and the ethyl acetate was removed under a reduced pressure to obtain Latex Dispersions (I'), (II'), (XVII'), (III'), (VII'), (a'), (b'), (c') and (d'), respectively. Each of the latex dispersions of these oleophilic magenta polymer couplers containing  $5.6 \times 10^{-3}$  mol of the coupler unit was mixed with 100 g of a silver halide emulsion containing  $5.6 \times 10^{-2}$  mol of silver iodobromide and 8 g of gelatin, and to the mixture was added 8 ml of a 4% acetone solution of 2-hydroxy-4,6-dichloro-s-triazine sodium salt. After adjusting the pH to 6.5, the emulsion was coated on a cellulose triacetate support having a subbing layer to prepare Samples 1 to 9.

These films were exposed stepwise for sensitometry and then subjected to the following color development processing.

| Color Development Processing Step | Time         | Temperature (°C.) |
|-----------------------------------|--------------|-------------------|
| 1. Color development              | 3 min 15 sec | 38                |
| 2. Bleaching                      | 6 min 30 sec | "                 |
| 3. Washing with water             | 2 min        | "                 |
| 4. Fixing                         | 4 min        | "                 |
| 5. Washing with water             | 4 min        | "                 |

-continued

| Color Development Processing Step | Time  | Temperature (°C.) |
|-----------------------------------|-------|-------------------|
| 6. Stabilizing                    | 1 min | "                 |

5

The processing solutions used in the color development processing had the following compositions:

| Color Developer Solution                                |                      |
|---------------------------------------------------------|----------------------|
| Water                                                   | 800 ml               |
| 4-(N-Ethyl-N-hydroxyethyl)amino-2-methylaniline Sulfate | 5 g                  |
| Sodium Sulfite                                          | 5 g                  |
| Hydroxylamine Sulfate                                   | 2 g                  |
| Potassium Carbonate                                     | 30 g                 |
| Potassium Hydrogencarbonate                             | 1.2 g                |
| Potassium Bromide                                       | 1.2 g                |
| Sodium Chloride                                         | 0.2 g                |
| Trisodium Nitrotriacetate                               | 1.2 g                |
| Water to make                                           | 1 liter<br>(pH 10.1) |

  

| Bleaching Solution                              |                     |
|-------------------------------------------------|---------------------|
| Water                                           | 800 ml              |
| Iron (III) Ammonium Ethylenediaminetetraacetate | 100 g               |
| Disodium Ethylenediaminetetraacetate            | 10 g                |
| Potassium Bromide                               | 150 g               |
| Acetic Acid                                     | 10 g                |
| Water to make                                   | 1 liter<br>(pH 6.0) |

  

| Fixing Solution        |                     |
|------------------------|---------------------|
| Water                  | 800 ml              |
| Ammonium Thiosulfate   | 150 g               |
| Sodium Sulfite         | 10 g                |
| Sodium Hydrogensulfite | 2.5 g               |
| Water to make          | 1 liter<br>(pH 6.0) |

10

The photographic properties thus-obtained are shown in Table 1 below.

TABLE 1

| Sample                 | Latex Used | Fog  | Gamma | Relative Sensitivity | (*)<br>Maximum Color Density |
|------------------------|------------|------|-------|----------------------|------------------------------|
| 1. (Present Invention) | (I')       | 0.05 | 1.21  | 100                  | 1.25                         |
| 2. (Present Invention) | (II')      | 0.05 | 1.30  | 104                  | 1.34                         |
| 3. (Present Invention) | (XVII')    | 0.05 | 1.17  | 94                   | 1.19                         |
| 4. (Present Invention) | (III')     | 0.05 | 1.26  | 99                   | 1.30                         |
| 5. (Present Invention) | (VII')     | 0.05 | 1.35  | 106                  | 1.38                         |
| 6. (Comparison)        | (a')       | 0.05 | 0.53  | — <sup>(*)</sup>     | 0.61                         |
| 7. (Comparison)        | (b')       | 0.05 | 0.71  | 69                   | 0.85                         |
| 8. (Comparison)        | (c')       | 0.05 | 0.49  | — <sup>(*)</sup>     | 0.57                         |
| 9. (Comparison)        | (d')       | 0.06 | 0.55  | — <sup>(*)</sup>     | 0.65                         |

<sup>(\*)</sup>Relative value of a reciprocal of the exposure amount required for obtaining an optical density of fog value +0.2.

<sup>(\*)</sup>Relative sensitivity was not determined since the color density obtained was too low.

It is apparent from the results shown in Table 1 that Samples 1, 2, 3, 4 and 5 according to the present invention provide increased gamma, relative sensitivity, and maximum color density without an increase in fog in comparison with the Comparative Samples 6, 7, 8 and 9, and thus they are clearly advantageous with respect to the color forming property.

The comparative oleophilic magenta polymer coupler (a), (b), (c) and (d) have the following compositions.

30

40

(a)



-continued



(b)



(c)



(d)

## EXAMPLE 2

20 g of each of Oleophilic Polymer Couplers (XII), (XIV) and (XV) according to the present invention and Comparative Oleophilic Polymer Couplers (e), (f), (g) and (h) and was dissolved by heating in 80 ml of ethyl acetate and the solution was added to 400 ml of an 55 aqueous solution containing 20 g of gelatin and 1.2 g of sodium triisopropylnaphthalenesulfonate. The resulting mixture was dispersed using a colloid mill and the ethyl acetate was removed under a reduced pressure to obtain Latex Dispersions (XII'), (XIV'), (XV'), (e'), (f'), (g') 60 and (h'), respectively. Each of the latex dispersions of these oleophilic polymer couplers containing  $7.5 \times 10^{-3}$  mol of the coupler unit was mixed with 100 g of a silver halide emulsion containing  $8.4 \times 10^{-2}$  mol of silver iodobromide and 8 g of gelatin, to which 8 ml of 65 a 4% acetone solution of 2-hydroxy-4,6-dichloro-s-triazone sodium salt was added. The pH of the mixture was adjusted to 6.7 and the mixture was coated on a cellul-

lose triacetate film in an amount of silver coated of  $1.2 \times 10^{-3}$  mol/m<sup>2</sup>, to prepare Samples 10 to 16.

These films were exposed stepwise for sensitometry and then subjected to the following color development processing.

## Color Development Processing Step (38° C.)

Time  
(min)

- |                       |   |
|-----------------------|---|
| 1. First development  | 3 |
| 2. Washing with water | 1 |
| 3. Reversal           | 2 |
| 4. Color development  | 6 |
| 5. Control            | 2 |
| 6. Bleaching          | 6 |
| 7. Fixing             | 4 |
| 8. Washing with water | 4 |
| 9. Stabilizing        | 1 |
| 10. Drying            |   |

The processing solutions used in the color development processing had the following compositions:

| First Development Solution                                                   |         | Bleaching Solution |                                                                                                                                                                                                                                                                                                                                              |         |       |         |      |
|------------------------------------------------------------------------------|---------|--------------------|----------------------------------------------------------------------------------------------------------------------------------------------------------------------------------------------------------------------------------------------------------------------------------------------------------------------------------------------|---------|-------|---------|------|
| Water                                                                        | 800 ml  | 5                  | Water                                                                                                                                                                                                                                                                                                                                        | 800 ml  |       |         |      |
| Sodium Tetrapolyphosphate                                                    | 2.0 g   |                    | Sodium Ethylenediaminetetraacetate                                                                                                                                                                                                                                                                                                           | 2.0 g   |       |         |      |
| Sodium Hydrogensulfite                                                       | 8.0 g   |                    | Dihydrate                                                                                                                                                                                                                                                                                                                                    |         |       |         |      |
| Sodium Sulfite                                                               | 37.0 g  | 10                 | Ammonium Iron (II) Ethylenediamine-tetraacetate Dihydrate                                                                                                                                                                                                                                                                                    | 120.0 g |       |         |      |
| 1-Phenyl-3-pyrazolidone                                                      | 0.35 g  |                    | Potassium Bromide                                                                                                                                                                                                                                                                                                                            | 100.0 g |       |         |      |
| Hydroquinone                                                                 | 5.5 g   |                    | Water to make                                                                                                                                                                                                                                                                                                                                | 1 liter |       |         |      |
| Sodium Carbonate Monohydrate                                                 | 28.0 g  |                    |                                                                                                                                                                                                                                                                                                                                              |         |       |         |      |
| Potassium Bromide                                                            | 1.5 g   | 15                 |                                                                                                                                                                                                                                                                                                                                              |         |       |         |      |
| Potassium Iodide                                                             | 13.0 g  |                    |                                                                                                                                                                                                                                                                                                                                              |         |       |         |      |
| Sodium Thiocyanate                                                           | 1.4 g   |                    |                                                                                                                                                                                                                                                                                                                                              |         |       |         |      |
| Water to make                                                                | 1 liter |                    |                                                                                                                                                                                                                                                                                                                                              |         |       |         |      |
| Reversal Solution                                                            |         | Fixing Solution    |                                                                                                                                                                                                                                                                                                                                              |         |       |         |      |
| Water                                                                        | 800 ml  | 20                 | Water                                                                                                                                                                                                                                                                                                                                        | 800 ml  |       |         |      |
| Hexasodium Nitrilo-N,N,N-trimethylene Phosphonate                            | 3.0 g   |                    | Ammonium Thiosulfate                                                                                                                                                                                                                                                                                                                         | 80.0 g  |       |         |      |
| Stannous Chloride Dihydrate                                                  | 1.0 g   |                    | Sodium Sulfite                                                                                                                                                                                                                                                                                                                               | 5.0 g   |       |         |      |
| Sodium Hydroxide                                                             | 8.0 g   | 30                 | Sodium Hydrogensulfite                                                                                                                                                                                                                                                                                                                       | 5.0 g   |       |         |      |
| Glacial Acetic Acid                                                          | 15.0 ml |                    | Water to make                                                                                                                                                                                                                                                                                                                                | 1 liter |       |         |      |
| Water to make                                                                | 1 liter |                    |                                                                                                                                                                                                                                                                                                                                              |         |       |         |      |
| Color Development Solution                                                   |         | Stabilizing Bath   |                                                                                                                                                                                                                                                                                                                                              |         |       |         |      |
| Water                                                                        | 800 ml  | 35                 | Water                                                                                                                                                                                                                                                                                                                                        | 800 ml  |       |         |      |
| Sodium Tetrapolyphosphate                                                    | 2.0 g   |                    | Formalin (37 wt % formaldehyde)                                                                                                                                                                                                                                                                                                              | 5.0 ml  |       |         |      |
| Benzyl Alcohol                                                               | 5.0 ml  |                    | Fuji Drywel                                                                                                                                                                                                                                                                                                                                  | 5.0 ml  |       |         |      |
| Sodium Sulfite                                                               | 7.5 g   |                    | Water to make                                                                                                                                                                                                                                                                                                                                | 1 liter |       |         |      |
| Trisodium Phosphate (12 hydrate)                                             | 36.0 g  |                    |                                                                                                                                                                                                                                                                                                                                              |         |       |         |      |
| Potassium Bromide                                                            | 1.0 g   |                    |                                                                                                                                                                                                                                                                                                                                              |         |       |         |      |
| Potassium Iodide                                                             | 90.0 g  |                    |                                                                                                                                                                                                                                                                                                                                              |         |       |         |      |
| Sodium Hydroxide                                                             | 3.0 g   |                    |                                                                                                                                                                                                                                                                                                                                              |         |       |         |      |
| Citrazic Acid                                                                | 1.5 g   |                    |                                                                                                                                                                                                                                                                                                                                              |         |       |         |      |
| 4-Amino-3-methyl-N—ethyl-N—(β-hydroxyethyl)aniline Sesquisulfate Monohydrate | 11.0 g  |                    |                                                                                                                                                                                                                                                                                                                                              |         |       |         |      |
| Ethylenediamine                                                              | 3.0 g   |                    |                                                                                                                                                                                                                                                                                                                                              |         |       |         |      |
| Water to make                                                                | 1 liter |                    |                                                                                                                                                                                                                                                                                                                                              |         |       |         |      |
| Control Solution                                                             |         | TABLE 2            |                                                                                                                                                                                                                                                                                                                                              |         |       |         |      |
| Water                                                                        | 800 ml  | 40                 | Maximum                                                                                                                                                                                                                                                                                                                                      |         |       |         |      |
| Glacial Acetic Acid                                                          | 5.0 ml  |                    | Latex                                                                                                                                                                                                                                                                                                                                        |         |       |         |      |
| Sodium Hydroxide                                                             | 3.0 g   |                    | Sample                                                                                                                                                                                                                                                                                                                                       |         | Fog   | Color   |      |
| Dimethylaminoethaneisothiourea                                               | 1.0 g   | 45                 | Used                                                                                                                                                                                                                                                                                                                                         |         | Gamma | Density |      |
| Dihydrochloride                                                              |         |                    | 10. (Present Invention)                                                                                                                                                                                                                                                                                                                      | (XII')  | 0.03  | 1.17    | 1.24 |
| Water to make                                                                | 1 liter |                    | 11. (Present Invention)                                                                                                                                                                                                                                                                                                                      | (XIV')  | 0.03  | 1.15    | 1.21 |
|                                                                              |         |                    | 12. (Present Invention)                                                                                                                                                                                                                                                                                                                      | (XV')   | 0.03  | 1.26    | 1.27 |
|                                                                              |         | 50                 | 13. (Comparison)                                                                                                                                                                                                                                                                                                                             | (e')    | 0.02  | 0.49    | 0.62 |
|                                                                              |         |                    | 14. (Comparison)                                                                                                                                                                                                                                                                                                                             | (f')    | 0.03  | 0.71    | 0.95 |
|                                                                              |         |                    | 15. (Comparison)                                                                                                                                                                                                                                                                                                                             | (g')    | 0.03  | 0.85    | 1.01 |
|                                                                              |         |                    | 16. (Comparison)                                                                                                                                                                                                                                                                                                                             | (h')    | 0.03  | 0.73    | 0.90 |
|                                                                              |         | 55                 | It is apparent from the results shown in Table 2 that Samples 10, 11 and 12 according to the present invention provide increased gamma and maximum color density without an increase in fog in comparison with the Comparative Samples 13, 14, 15 and 16, and thus they are clearly advantageous with respect to the color forming property. |         |       |         |      |
|                                                                              |         | 60                 | 65 The comparative oleophilic magenta polymer couplers (e), (f), (g) and (h) have the following compositions.                                                                                                                                                                                                                                |         |       |         |      |



(e)



(f)



(g)



(h)

### EXAMPLE 3

A latex solution containing  $5.6 \times 10^{-3}$  mol of each of magenta polymer coupler latexes (S), (E), (T) and (F) according to the present invention and the comparative magenta polymer coupler latex (i) which was prepared by the synthesis method I and 30 ml of water were mixed with 100 g of a silver halide emulsion containing  $5.6 \times 10^{-2}$  mol of silver iodobromide and 8 g of gelatin,

and to the mixture was added 8 ml of a 4% acetone solution of 2-hydroxy-4,6-dichloro-s-triazine sodium salt. After adjusting the pH to 6.5, the emulsion was coated on a cellulose triacetate support having a subbing layer to prepare Samples 17 to 21.

These films were exposed stepwise for sensitometry and then subjected to the color development processing in the same manner as described in Example 1.

The photographic properties thus-obtained are shown in Table 3 below.

TABLE 3

| Sample                  | Latex Used | Fog  | Gamma | Maximum Color Density |
|-------------------------|------------|------|-------|-----------------------|
| 17. (Present Invention) | (S)        | 0.06 | 1.44  | 1.45                  |
| 18. (Present Invention) | (E)        | 0.05 | 1.36  | 1.38                  |
| 19. (Present Invention) | (T)        | 0.06 | 1.41  | 1.49                  |
| 20. (Present Invention) | (F)        | 0.05 | 1.30  | 1.35                  |
| 21. (Comparison)        | (i)        | 0.06 | 1.12  | 1.06                  |

It is apparent from the results shown in Table 3 that Samples 17, 18, 19 and 20 according to the present invention provide increased gamma and maximum color density without an increase in fog in comparison with the Comparative Sample 21, and thus they are clearly advantageous with respect to the color forming property.

The comparative magenta polymer coupler latex (i) has the following composition.



While the invention has been described in detail and with reference to specific embodiments thereof, it will be apparent to one skilled in the art that various changes and modifications can be made therein without departing from the spirit and scope thereof.

What is claimed is:

1. A silver halide color photographic light sensitive material comprising a support having thereon a silver halide emulsion layer containing a magenta color image forming polymer coupler latex which is capable of forming a dye upon coupling with an oxidation product of an aromatic primary amine developing agent and which is a polymer or copolymer having a repeating unit derived from a monomer represented by the following general formula (I):



wherein R<sub>1</sub> represents a hydrogen atom, a lower alkyl group containing from 1 to 4 carbon atoms or a chlorine atom; R<sub>2</sub> represents an unsubstituted or substituted alkylene group which may be a straight chain or a branched chain; R<sub>3</sub> represents an unsubstituted or substituted alkylene group which may be a straight chain or a branched chain, an unsubstituted or substituted phenyl group or an unsubstituted or substituted aralkylene group; X represents —CONH—, —NHCONH—, or —NHCOO—; Y represents —CONH— or —COO—; Z represents —O—, —S—, —SO—, —SO<sub>2</sub>—, —CONH— or —COO—; Ar represents an unsubstituted or substituted phenyl group; l represents 0 or 1; m represents 0 or 1; and n represents 0 or 1.

lene group or an unsubstituted or substituted aralkylene group; X represents —CONH—, —NHCONH—, or —NHCOO—; Y represents —CONH— or —COO—; Z represents —O—, —S—, —SO—, —SO<sub>2</sub>—, —CONH— or —COO—; Ar represents an unsubstituted or substituted phenyl group; l represents 0 or 1; m represents 0 or 1; and n represents 0 or 1.

2. A silver halide color photographic light-sensitive material as claimed in claim 1, wherein the alkylene group represented by R<sub>2</sub> is an alkylene group having from 1 to 10 carbon atoms.

3. A silver halide color photographic light-sensitive material as claimed in claim 1, wherein the alkylene group represented by R<sub>3</sub> is an alkylene group having from 1 to 10 carbon atoms.

4. A silver halide color photographic light-sensitive material as claimed in claim 1, wherein the substituent for the substituted alkylene group, the substituted phenylene group or the substituted aralkylene group represented by R<sub>2</sub> or R<sub>3</sub> is an aryl group, a nitro group, a hydroxy group, a cyano group, a sulfo group, an alkoxy group, an aryloxy group, an acyloxy group, an acylamino group, a sulfonamido group, a sulfamoyl group, a halogen atom, a carboxy group, a carbamoyl group, an alkoxycarbonyl group or a sulfonyl group.

(i)

5. A silver halide color photographic light-sensitive material as claimed in claim 1, wherein the substituent for the substituted phenyl group represented by Ar is an alkyl group, an alkoxy group, an aryloxy group, an alkoxycarbonyl group, an acylamino group, a carbamoyl group, an alkylcarbamoyl group, a dialkylcarbamoyl group, an arylcarbamoyl group, an alkylsulfonyl group, an arylsulfonyl group, an alkylsulfonamido group, an arylsulfonamido group, a sulfamoyl group, an alkylsulfamoyl group, a dialkylsulfamoyl group, an alkylthio group, an arylthio group, a cyano group, a nitro group, or a halogen atom.

6. A silver halide color photographic light-sensitive material as claimed in claim 1, wherein the substituent for the substituted phenyl group represented by Ar is a halogen atom, an alkyl group, an alkoxy group, an alkoxycarbonyl group, or a cyano group.

7. A silver halide color photographic light-sensitive material as claimed in claim 1, wherein the substituted phenyl group represented by Ar is a phenyl group represented by the following general formula (III):



wherein R<sub>4</sub>, which is present at the 4-position or 5-position of the phenyl group, represents a halogen atom, an acylamino group, a carbamoyl group, a sulfonyl group, a sulfonamido group, a cyano group or an alkoxy carbonyl group.

8. A silver halide color photographic light-sensitive material as claimed in claim 7, wherein R<sub>4</sub> is a halogen atom.

9. A silver halide color photographic light-sensitive material as claimed in claim 1, wherein the polymer is a homopolymer.

10. A silver halide color photographic light-sensitive material as claimed in claim 1, wherein the polymer is a copolymer.

11. A silver halide color photographic light-sensitive material as claimed in claim 10, wherein the copolymer contains a repeating unit derived from a non-color forming monomer which does not couple with the oxidation product of an aromatic primary amine developing agent.

12. A silver halide color photographic light-sensitive material as claimed in claim 11, wherein the non-color forming monomer is selected from the group consisting of an acrylic acid ester, an acrylic acid amide, a vinyl ester, an acrylonitrile, an aromatic vinyl compound, itaconic acid, citraconic acid, crotomic acid, vinylidene chloride, a vinyl alkyl ether, an ester of maleic acid, N-vinyl-2-pyrrolidone, N-vinyl pyridine, and 2- or 4-vinyl pyridine.

13. A silver halide color photographic light-sensitive material as claimed in claim 11, wherein the non-color forming monomer is selected from the group consisting of an acrylic acid ester, a methacrylic acid ester and a maleic acid ester.

14. A silver halide color photographic light-sensitive material as claimed in claim 1, wherein the amount of the color forming portion in the polymer latex is from 5% to 80% by weight.

15. A silver halide color photographic light-sensitive material as claimed in claim 1, wherein the amount of the color forming portion in the polymer latex is from 20% to 70% by weight.

16. A silver halide color photographic light-sensitive material as claimed in claim 14, wherein the gram number of the polymer latex containing 1 mol of coupler monomer is from 250 to 3,000.

17. A silver halide color photographic light-sensitive material as claimed in claim 1, wherein the magenta color image forming polymer coupler latex is a latex prepared by emulsion polymerization of a monomer

comprising a monomer coupler represented by the general formula (I).

18. A silver halide color photographic light-sensitive material as claimed in claim 1, wherein the magenta color image forming polymer coupler latex is a latex prepared by dissolving an oleophilic polymer coupler obtained by polymerization of a monomer comprising a monomer coupler represented by the general formula (I) in an organic solvent and then dispersing the solution in a latex form in an aqueous gelatin solution.

19. A silver halide color photographic light-sensitive material as claimed in claim 1, wherein the silver halide emulsion layer containing a magenta color image forming polymer coupler latex is a green-sensitive silver halide emulsion layer.

20. A silver halide color photographic light-sensitive material as claimed in claim 19, wherein the photographic light-sensitive material further comprises a blue-sensitive silver halide emulsion layer containing a yellow color image forming coupler and a red-sensitive silver halide emulsion layer containing a cyan color image forming coupler.

21. A method of forming a color image comprising developing an imagewise exposed silver halide color photographic light-sensitive material comprising a support having thereon a silver halide emulsion layer containing a magenta color image forming polymer coupler latex which is capable of forming a dye upon coupling with an oxidation product of an aromatic primary amine developing agent and which is a polymer or copolymer having a repeating unit derived from a monomer represented by the following general formula (I):



wherein R<sub>1</sub> represents a hydrogen atom, a lower alkyl group containing from 1 to 4 carbon atoms or a chlorine atom; R<sub>2</sub> represents an unsubstituted or substituted alkylene group which may be a straight chain or a branched chain; R<sub>3</sub> represents an unsubstituted or substituted alkylene group which may be a straight chain or a branched chain, an unsubstituted or substituted phenylene group or an unsubstituted or substituted aralkylene group; X represents  $\text{--CONH--}$ ,  $\text{--NHCONH--}$  or  $\text{--NHCOO--}$ ; Y represents  $\text{--CONH--}$  or  $\text{--COO--}$ ; Z represents  $\text{--O--}$ ,  $\text{--S--}$ ,  $\text{--SO--}$ ,  $\text{--SO}_2--$ ,  $\text{--CONH--}$  or  $\text{--COO--}$ ; Ar represents an unsubstituted or substituted phenyl group; l represents 0 or 1; m represents 0 or 1; and n represents 0 or 1; wherein said developing is conducted using an alkaline aqueous solution containing an aromatic primary amine developing agent.

\* \* \* \* \*